

## UNITED STATES PATENT OFFICE.

HOWARD CHARLES FUELLER, OF JACKSONVILLE, FLORIDA.

## PROCESS OF TREATING VEGETABLE FIBER.

No Drawing. Application filed July 12, 1919, Serial No. 310,431. Renewed November 29, 1922.

*To all whom it may concern:*

Be it known that I, HOWARD CHARLES FUELLER, a citizen of the United States, and a resident of Jacksonville, in the county of 5 Duval and State of Florida, have invented certain new and useful Improvements in a Process of Treating Vegetable Fiber, of which the following is a specification.

My invention is an improvement in a process of treating vegetable fiber, and has for its object to provide a new and improved process of the character specified, for preparing Florida or Spanish moss and the like for use as a stuffing for mattresses, 15 cushions and the like, wherein the moss is dehydrated then dyed and afterwards stiffened and glossed.

In the present method, the green moss is subjected to four steps or treatments, the 20 first being treating with an acid, the second treating with an alkali, the third dyeing, and the fourth stiffening and glossing.

In carrying out this process, I first subject the green moss to a bath of acid, which 25 acts to draw out the vegetable juices. The moss is left in this acid bath from one to three hours, in accordance with the condition of the moss, that is whether the moss is green or partly cured or dried. The moss 30 is then placed in the alkali bath, where it is treated for from fifteen to thirty minutes.

A preferable formula for the alkaline bath is a 2% solution of caustic soda, this chemical being preferable because of its low cost, 35 although any other alkali will answer equally well. After treatment in the alkaline bath, the moss is dried in a dryer, at a temperature of from 180° to 200° F. When dry it is dyed, by placing it in a bath of 40 dye stuff.

This dye bath may be composed of any suitable tannin containing material, as for instance log wood extract 10% to 15%, quercitron extract, 3%, and copperas 5%. 45 The moss treated by the acid and alkali is placed in the bath of dye stuff and kept for from one to two hours, that is until a good black is produced.

After the dye bath the moss is subjected 50 to treatment for stiffening and glossing the same; as for instance coating with gelatine or glue. A preferable formula for this stiffening and glossing bath is glue two to four parts, water ten gallons, the amount of 55 glue being regulated in accordance with the degree of stiffness required. A certain

amount of 40% formaldehyde solution is added to the stiffening bath, and a soluble oil, such for instance as Turkey red oil, the formaldehyde serving as an antiseptic and 60 coating on the fiber while the oil gives a gloss and a soft feel to the moss.

Moss treated in the above manner may be prepared for use within a very short time, where ordinarily several weeks are necessary to cure the moss, that is to dry it in the 65 sun. Furthermore sun drying does not drive out the vegetable juices, and until they are removed the fiber cannot be dyed satisfactorily. 70

I have also found that the moss may be cured satisfactorily, merely by the use of an alkali, thus preparing the moss suitable for drying in one step instead of two. This 75 however requires greater time than treating with acid and alkali baths. In curing the moss as above mentioned, it is piled up and wetted down with an alkali, as for instance a solution of caustic soda, or soda ash. The pile is then left for a week, after which it is 80 turned over and again wetted if too dry and is left for another week.

This wetting with the alkali causes the moss to heat, and cures the same. In the center of the pile, the moss becomes hot 85 enough to cook an egg, too hot to handle with the hands. This moss so treated may be at once dyed and treated with the stiffening and glossing bath.

Vegetable fiber treated as above mentioned serves all the purposes of hair, as for instance stuffing of mattresses, cushions, automobile seats and the like. The product has the resiliency of hair, it is sanitary and practically indestructible. The formaldehyde produces with the glue or gelatine an insoluble compound, which produces an insoluble coating on the fiber. When this coating is dried by heat at about 180° F., the fiber is given a nice curl, and it is moisture 100 proof. Sulphuric acid in a 4% solution may be used for the acid bath. The purpose of the alkali after the acid bath, is to neutralize the acid.

It will be understood that copper sulphite 105 or any other suitable mordant may be used if desired.

In the acid bath a preferable mixture is one hundred eighty-six pounds of sulphuric acid, 66° B., in five hundred gallons of water. 110

In the stiffening bath a preferable mix-

ture is one and a half to three pounds of glue to the gallon of water, (the amount depending upon the grade of glue, whether hide or bone glue). To this I add from one-half to one gallon of so-called 40% formaldehyde solution, to each five hundred gallons of the above mixture. Estimating the formaldehyde solution at eight pounds to the gallon, four to eight pounds will be used in the five hundred gallons. The soluble oil added to the stiffening bath retards or modifies the action of the formaldehyde.

For the alkaline bath a preferable formula is eighty-one and one-quarter pounds of caustic soda, 76% to five hundred gallons of water.

I claim:

1. A process of treating vegetable fiber, as for instance Spanish moss, which consists in the chemical removal of the plant juices from the fiber, the dyeing of the fiber, and the treatment of the fiber with a solution for stiffening and glossing the same, the chemical removal of the plant juices consisting in

subjecting the fiber to acid and alkaline baths.

2. A process of treating vegetable fiber, as for instance Spanish moss, which consists in the chemical removal of the plant juices from the fiber, the dyeing of the fiber, and the treatment of the fiber with a solution for stiffening and glossing the same, the means for stiffening and glossing the fiber consisting of a solution of glue, formaldehyde and soluble oil.

3. A process of preparing vegetable fiber for use as a stuffing material for mattresses and the like, which consists in the chemical removal of plant juices from the fiber, in the dyeing of the fiber, and in treating the fiber with a solution for stiffening and glossing the same.

4. A process of treating vegetable fiber which consists in removing the plant juices from the fiber with acid, neutralizing the acid, dyeing the fiber, and treating it with an insoluble gluey coating.

HOWARD CHARLES FUELLER.